

1

2,991,251

## CORROSION INHIBITING LUBRICATING COMPOSITION

Harry W. Rudel, Roselle, and William Seitz, Union, N.J., assignors to Esso Research and Engineering Company, a corporation of Delaware  
No Drawing. Filed Sept. 27, 1957, Ser. No. 686,598  
5 Claims. (Cl. 252—47.5)

This invention relates to materials and methods for inhibiting the lead corroding tendency of compositions containing partial esters of aliphatic polyhydroxy alcohols. Particularly, it relates to oil compositions comprising partial esters of polyhydroxy alcohols and minor amounts, sufficient to inhibit lead corrosion, of mercaptobenzothiazole or its derivatives and/or hydroxy benzoic acid or its derivatives.

Fatty acid partial esters of aliphatic polyhydric alcohols, e.g., sorbitan monooleate, have found widespread use for inhibiting the corrosion of iron. However, in certain applications where the composition containing the partial ester also comes in contact with lead, the partial ester causes excessive corrosion of lead, even though inhibiting the corrosion of iron. For example, mineral oil compositions containing sorbitan monooleate have been used in the crankcase of piston-type aircraft engines to prevent rusting during storage. For this use, the engine is run for a short period of time to circulate the composition through the engine, after which the engine is turned off, and the oil drains back to the crankcase, leaving a protective film on the cylinder walls and other internal parts of the engine. Recently, for purposes of economy, it has become desirable to use the same composition for actual operation of the engine, rather than to remove the rust preventive oil composition and replace it with fresh lubricating oil. However, when the oil composition containing the partial ester was later used as lubricating oil, such that the composition was circulated through the engine for long periods of time, excessive corrosion of the lead in the copper-lead bearings in the engine occurred. It has now been found that the lead corroding tendencies of these partial esters may be effectively curbed, without interfering with their rust inhibiting properties, by the addition of a minor amount of mercaptobenzothiazole and its derivatives, or hydroxy benzoic acid and its derivatives.

The compositions of the invention will generally comprise an oil base, about 1 to 25, e.g., 2 to 10 weight percent of the partial ester, and about 0.01 to 2.0, e.g., 0.03 to 1.0 weight percent of the lead corrosion inhibiting material.

The oil base will generally be a mineral lubricating oil, although other petroleum bases such as kerosene, gas oil, naphthas, petrolatum, etc. may be used.

The partial esters used as rust preventives include the C<sub>12</sub> to C<sub>22</sub> fatty acid partial esters of aliphatic polyhydric alcohols having about 3 to 12, e.g., 3 to 8 carbon atoms, and about 2 to 8, e.g., 3 to 6 hydroxy groups per molecule. Preferred materials are the mono- and diesters of C<sub>3</sub> to C<sub>6</sub> alcohols having about 3 to 6 hydroxyl groups and prepared from C<sub>12</sub> to C<sub>18</sub> fatty acids. The above type of partial esters includes the partial esters of the mono-dehydrated aliphatic polyhydric alcohols, which are well known in the art, for example, see U.S. Patent 2,434,490, as well as partial esters of non-dehydrated aliphatic polyhydric alcohols, e.g. pentaerythritol monooleate.

Specific examples of the above types of partial esters will therefore include: glyceryl monooleate, pentaerythritol monooleate, sorbitan monooleate, the dioleates of sorbitan, mannan, pentaerythritol and related polyhydric alcohols, the corresponding partial stearic and palmitic

2

acid esters of these alcohols, and partial esters of these alcohols made from mixtures of these fatty acids.

The lead corrosion inhibiting agents are organic materials containing an aromatic nucleus, and are of two general types as follows:

Mercaptobenzothiazoles and its derivatives having the general formula:



15 wherein each R is hydrogen or a C<sub>1</sub> to C<sub>8</sub>, e.g., C<sub>1</sub> to C<sub>4</sub> alkyl group. Specific examples of such materials include: 2-mercaptobenzothiazole; 2-mercaptop, 4,6-dimethyl benzothiazole; 2-mercaptop, 4-methyl, 6-octyl benzothiazole; 2-mercaptop, 4-tertiary butyl benzothiazole; etc.

20 Salicylic acid and its derivatives having the general formula:



30 wherein R is hydrogen or a C<sub>1</sub> to C<sub>8</sub> straight or branched-chain alkyl group.

35 Specific examples of the salicylic acid materials of the above formulas include: salicylic acid, 2-hydroxy-3-methyl benzoic acid, 2-hydroxy-4 octyl benzoic acid, etc.

40 Other additive materials, to adapt the composition of the invention to special applications, may also be included in the composition in amounts of about 0.05 to 10.0 wt. percent based on the weight of the total composition. For example, it may be desirable to add other rust preventive additives, such as petroleum sulfonates and lecithin; viscosity index improvers, such as polymethacrylates and polyisobutylene; oxidation inhibitors; etc. Materials of increased consistency may also be prepared by thickening the oil composition of the invention with appropriate soaps, polymers, waxes, etc. In some cases, the addition of a C<sub>1</sub> to C<sub>18</sub>, e.g. C<sub>2</sub> to C<sub>8</sub>, alkyl amine to the composition seems to aid in inhibiting lead corrosion, particularly when it is used in conjunction with the salicylic acid type inhibitor.

45 The lead corrosion inhibitors of the invention were found to be the only effective materials of a wide number of similar type materials and other known inhibiting agents which were tested. This is shown by the following examples:

### EXAMPLE I

50 The test for lead corrosion was the S.O.D. lead corrosion test, which was carried out by suspending rotating copper and lead strips for one hour in the oil composition maintained at a temperature of 325° F. Following this, the lead strip was removed and the change in weight of the strip, in terms of milligrams per square inch of strip, was measured. The above test was carried out on: the base oil per se, which was a solvent extracted Mid-Continent mineral lubricating oil having a viscosity of 100 SUS at 210° F.; a composition consisting of 95 weight percent of the base oil and 5 weight percent of a commercial sorbitan monooleate sold under the trade name of Span 80; and the oil-sorbitan monooleate composition containing various different additives. The re-

sults of this series of tests are summarized in the following table:

Table I

S.O.D. LEAD CORROSION TEST  
[1 hour at 325° F. with copper catalyst]

| Wt. Percent Inhibitor Added to Oil-Sorbitan Monooleate Composition | Lead Strip Weight Loss (mg./sq. in.) |
|--------------------------------------------------------------------|--------------------------------------|
| Oil, per se.....                                                   | 6                                    |
| 95% oil and 5% sorbitan monooleate.....                            | 249                                  |
| 1.0 Diteriary butyl para cresol.....                               | 231                                  |
| 1.0 Phenyl alpha naphthylamine.....                                | 262                                  |
| 1.0 Hydroquinone monomethyl ether.....                             | 308                                  |
| 1.0 Lecithin.....                                                  | 395                                  |
| 1.0 Amine from hydrogenated tallow acids.....                      | 194                                  |
| 0.5 2-Ethyl hexyl amine.....                                       | 195                                  |
| 1.0 adduct of salicyaldehyde and ethylene diamine.....             | 361                                  |
| 0.5 Diocetyl phosphoric acid.....                                  | 268                                  |
| 0.5 Tricetyl phosphate.....                                        | 187                                  |
| 0.5 Zinc diocetyl dithiophosphate.....                             | 278                                  |
| 1.0 Cetyl mercaptan.....                                           | 312                                  |
| 0.5 Tridodecyl borate.....                                         | 308                                  |
| 0.5 Methyl thiram disulfide.....                                   | 207                                  |
| 1.0 Phenothiazine.....                                             | 199                                  |
| 1.0 Mercaptobenzothiazole.....                                     | +4                                   |
| 0.1 Mercaptobenzothiazole.....                                     | 132                                  |

As seen from the above tests, the base oil per se showed a lead strip weight loss of only 6 mg., yet when 5 weight percent of sorbitan monooleate was added to this oil, it then gave a weight loss of 249 mg. Of the numerous inhibitors tested above, it is seen that only the mercaptobenzothiazole was effective. Thus, one weight percent of mercaptobenzothiazole had actually resulted in a small gain of +4 mg., and as little as one-tenth of 1 percent of mercaptobenzothiazole had effectively reduced the corrosivity about in half.

## EXAMPLE II

Another series of compositions was tested by adding various inhibitors to the oil-sorbitan monooleate composition of Example I. However, in these tests the lead strip was exposed for two hours at 325° F. and no copper was present. Results are reported in Table II.

Table II  
MODIFIED S.O.D. LEAD CORROSION TEST  
[2 hrs. at 325° F. without copper catalyst]

| Wt. Percent Inhibitor Added to Oil-sorbitan Monooleate Composition | Weight Loss of Lead Test Strip (mg./sq. in.) |
|--------------------------------------------------------------------|----------------------------------------------|
| 95% oil and 5% sorbitan monooleate.....                            | 121                                          |
| 0.1 Salicylic acid.....                                            | 10                                           |
| 0.05 Salicylic acid.....                                           | 100                                          |
| 0.1 Salicylic acid+0.1 n-butyl amine.....                          | 5                                            |
| 0.05 Salicylic acid+0.05 n-butyl amine.....                        | 101                                          |
| 0.1 Salicylic acid+0.05 mercaptobenzothiazole.....                 | 18                                           |
| 0.05 Salicylic acid+0.05 mercaptobenzothiazole.....                | 63                                           |

As seen from Table II, the lead corrosiveness of the oil-sorbitan monooleate composition was somewhat less in the absence of the copper catalyst (cf. Table I). The salicylic acid per se was very effective in inhibiting the lead corrosion. The addition of 0.1% alkyl amine with the 0.1% salicylic acid was also found very effective,

as are blends of salicylic acid and mercaptobenzothiazole. The use of aliphatic hydroxy acids such as citric, maleic and tartaric acids was not effective.

The inhibitors of the invention can also be mixed directly with the partial ester or concentrates thereof to form a rust preventive additive mixture which is also inhibited against lead corrosion.

To further illustrate the invention, other compositions can be prepared as follows:

- 10 A. 0.05 wt. percent of 4-methyl, 6-n-octyl benzothiazole can be added by simple mixing to a composition consisting of 1.0 wt. percent of glyceryl monostearate and 99.0 wt. percent of mineral lubricating oil of the type used in Example I.
- 15 B. 2.0 wt. percent of 2-hydroxy-4-n-octyl benzoic acid can be added by simple mixing to a composition consisting of 10.0 wt. percent of the dioleate of manitan and 90.0 wt. percent of mineral lubricating oil of the type used in Example I.
- 20 C. 5 wt. percent of mercaptobenzothiazole may be mixed with 95 wt. percent of Span 80 (sorbitan monooleate) to form an additive mixture.

In summary, the invention relates to materials and methods for inhibiting the lead corroding tendencies of compositions containing a fatty acid partial ester (usually the mono- or diester) of a polyhydric alcohol by mixing into said compositions about 2 to 40 wt. percent, e.g. 4 to 20 wt. percent, based on the weight of partial ester, a lead corrosion inhibitor. This lead corrosion inhibitor may be mercaptobenzothiazole, or its ring substituted alkyl derivatives or salicylic acid or its ring substituted alkyl derivatives or mixtures thereof.

What is claimed is:

1. A lubricating composition which is rust preventive and substantially non-corrosive to lead, which comprises a major proportion of mineral lubricating oil, about 1 to 25 wt. percent of sorbitan monooleate, and about .03 to 1.0 wt. percent of a material selected from the group consisting of mercaptobenzothiazole, salicylic acid, and mixtures thereof.
2. The lubricating composition of claim 1, wherein said material is mercaptobenzothiazole.
3. The lubricating composition of claim 1, wherein said material is salicylic acid.
4. The lubricating composition of claim 1 which also contains 0.5 to 10.0 wt. percent of a  $C_1$  to  $C_{18}$  alkyl amine.
5. A lubricating composition which is rust preventive and substantially non-corrosive to lead, comprising a major amount of mineral lubricating oil, about 2 to 10 wt. percent of sorbitan monooleate, and about 0.03 to 1.0 wt. percent of a material selected from the group consisting of mercaptobenzothiazole and salicylic acid.

## 55 References Cited in the file of this patent

## UNITED STATES PATENTS

- 2,154,097 Loane ..... Apr. 11, 1939  
2,366,074 Wasson et al. ..... Dec. 26, 1944  
60 2,482,517 Schiermeir ..... Sept. 20, 1949